

# United States Patent [19]

Watarai et al.

[11] 3,895,945

[45] July 22, 1975

[54] **PROCESS FOR PREPARATION OF A  
DYESTUFF SENSITIZED  
PHOTOCONDUCTIVE COMPOSITION**

[75] Inventors: **Syu Watarai; Yoshio Seoka**, both of  
Tokyo, Japan

[73] Assignee: **Rank Xerox, Ltd.**, London, England

[22] Filed: **Nov. 14, 1973**

[21] Appl. No.: **415,594**

[52] U.S. Cl. .... **96/1.6; 96/1.5; 260/67.5;  
260/315; 260/895**

## OTHER PUBLICATIONS

J. Chem. Soc. 117:1542-1550 (1920) Copisarow.

Primary Examiner—Henry R. Jiles  
Assistant Examiner—S. D. Winters  
Attorney, Agent, or Firm—James J. Ralabate; James P.  
O'Sullivan; John H. Faro

[57]

## ABSTRACT

Process for preparation of polymeric dyestuffs of the  
formula:



[51] Int. Cl. .... **G03g 5/06; G03c 1/72**

[58] Field of Search..... **260/315, 67.5, 895;  
96/1.5, 1.6, 1.5 C**

[56] **References Cited**

### UNITED STATES PATENTS

3,647,432 3/1972 Holstead ..... 260/315

wherein

R is alkyl of 1 to about 5 carbon atoms; and  
X is an anion residue.

Such polymeric materials are highly effective sensitizers  
for organic photoconductors such as the poly(-  
vinylcarbazoles).

**11 Claims, No Drawings**

**PROCESS FOR PREPARATION OF A DYESTUFF  
SENSITIZED PHOTOCONDUCTIVE  
COMPOSITION**

**BACKGROUND OF THE INVENTION**

**1. Field of the Invention**

This invention relates to a process for preparation of electrophotographic sensitizers. More specifically, this invention involves a process for the preparation of polymeric triaryl methane dyestuffs. These dyestuffs are highly effective in the sensitization of organic photoconductive materials.

**2. Description of the Prior Art**

The formation and development of images on the imaging surfaces of photoconductive materials by electrostatic means is well-known. The best known of the commercial processes, more commonly known as xerography, involves forming a latent electrostatic image on the imaging surface of an imaging member by first uniformly electrostatically charging the surface of the imaging layer in the dark and then exposing this electrostatically charged surface to a light and shadow image. The light struck areas of the imaging layer are thus rendered conductive and the electrostatic charge selectively dissipated in these irradiated areas. After the photoconductor is exposed, the latent electrostatic image on this image bearing surface is rendered visible by development with a finely divided colored electroscopic material, known in the art as "toner." This toner will be principally attracted to those areas on the image bearing surface which retain the electrostatic charge and thus form a visible powder image.

The developed image can then be read or permanently affixed to the photoconductor where the imaging layer is not to be reused. This latter practice is usually followed with respect to the binder-type photoconductive films (e.g. zinc oxide/insulating resin) where the photoconductive imaging layer is also an integral part of the finished copy.

In so-called "plain paper" copying systems, the latent image can be developed on the imaging surface of a reusable photoconductor or transferred to another surface, such as a sheet of paper, and thereafter developed. When the latent image is developed on the imaging surface of a reusable photoconductor, it is subsequently transferred to another substrate and then permanently affixed thereto. Any one of a variety of well-known techniques can be used to permanently affix the toner image to the copy sheet, including overcoating with transparent films, and solvent or thermal fusion of the toner particles to the supportive substrate.

In the above plain paper copying system, the materials used in the photoconductor layer should preferably be capable of rapid switching from insulative to conductive to insulative state in order to permit cyclic use of the imaging layer. The failure of a material to return to its relatively insulative state prior to the succeeding charging sequence will result in an increase in the dark decay rate of the photoconductor. This phenomenon, commonly referred to in the art as "fatigue" has in the past been avoided by the selection of photoconductive materials possessing rapid switching capacity. Typical of the materials suitable for use in such a rapidly cycling imaging system include anthracene, sulfur, selenium and mixtures thereof (U.S. Pat. No. 2,297,691), selenium being preferred because of its superior photosensitivity.

In addition to anthracene, other organic photoconductive materials, most notably, poly(N-vinylcarbazole), have been the focus of increasing interest in electrophotography, U.S. Pat. No. 3,037,861. Until recently, neither of these organic materials, namely anthracene or poly(N-vinylcarbazole), have received serious consideration as an alternative to such inorganic photoconductors as selenium, due to fabrication difficulties and/or the relative lack of speed and photosensitivity. The recent discovery that high loadings of 2,4,7-trinitro-9-fluoronone in polyvinylcarbazoles dramatically improves the photoresponsiveness of these materials has lead to a resurgence in interest in organic photoconductive materials, U.S. Pat. No. 3,484,237. Unfortunately, the inclusion of high loadings of such activators can and usually does result in phase separation of the various materials within such a composition. Thus, there will occur within such traditionally sensitized compositions, regions having in excessive activator regions deficient in activator and regions having the proper stoichiometric relationship of activator to photoconductor. The maximum amount of activator that may be added to most polymeric photoconductive materials without occasioning such phase separation generally will not exceed in excess of about 6 to about 8 weight percent.

One method suggested for avoiding the problems inherent in the use of such activators in conjunction with polymeric photoconductors, is the direct incorporation of these activators into the polymeric backbone of the photoconductor, U.S. Pat. No. 3,418,116. In this patent is disclosed the copolymerization of a vinyl monomer having an aromatic and/or heterocyclic substituent capable of an electron donor function with a vinyl monomer having an aromatic and/or heterocyclic substituent capable of an electron acceptor function. The spatial constraint placed upon these centers of differing electron density favors their charge transfer interaction upon photoexcitation of such a composition. These so-called "intramolecular" charge transfer complexes, more accurately designated "intrachain" charge transfer are believed to function substantially the same as charge transfer complexes formed between small activator molecules and a photoconductive polymer. The fact that the electron donor function and an electron acceptor are on a common polymeric backbone does not apparently change the  $\pi - \pi$  charge transfer interaction but merely increases the probability of it occurring. Unfortunately, the preparation of such copolymers from vinyl monomers having electron donor centers and vinyl monomers having an electron acceptor center is often beset with difficulty.

Separate and distinct from the sensitization of photoconductive materials with so-called "activator" materials is the addition of highly colored materials (dyestuffs) to photoconductive materials for the purpose of extending the spectral range of sensitivity of the photoconductors. The same problems and limitations discussed previously with regard to the inclusion of the activators into the photoconductive materials also applies with regard to the inclusion of dyestuffs into photoconductive materials. Traditionally, such dyestuffs are prepared independent of the photoconductive material and thereafter incorporated therein.

Carbazole functional dyestuffs have been previously disclosed in the technical literature, M. Copisarow, J. Chem. Soc. 117, 1542 - 1550 (1920). The Copisarow

article teaches the preparation of carbazole - blue and carbazole - violet dyestuff pigment. The author regards his process as a combination of the "aldehyde" and "phosgene" processes used in the formation of the triphenylamine series of dyes.

Traditionally, where the dyestuff is prepared independant of the photoconductive material, and thereafter dispersed therein the amount of dyestuff capable of incorporation into said photoconductor is limited.

It is, therefore, the object of this invention to enhance the sensitization of organic photoconductive materials.

Another object of this invention is to provide a process which enables the incorporation of relatively large concentrations of dyestuffs into photoconductive materials without adversely altering the physical properties of said photoconductive materials.

A further object of this invention is to provide a process for preparation of dyestuffs.

Yet a further object of this invention is to provide a process for the preparation of dyestuffs whereby the association of said dyestuff with an organic photoconductive material is enhanced.

#### SUMMARY OF THE INVENTION

The above and related objects are achieved by providing a process for the preparation of a triaryl methane dyestuff wherein a mixture containing an organic polymeric photoconductive material; about 2 to about 50 parts by weight N-alkyl-3-formylcarbazole per 100 parts organic polymeric photoconductive material and a quantity of polyphosphoric acid equivalent to about 5 to about 50 times the weight of organic polymeric photoconductive material, is heated with agitation at a temperature ranging from about 20 to about 120°C for a period sufficient to effect formation of the desired dyestuff. The temperature at which such reaction is carried out will, of course, determine the rate at which such dyestuff is formed. It is also noteworthy that in the dyestuff formation process, the reaction may be terminated prior to complete polymerization of the N-alkyl-3-formylcarbazole. In the preferred embodiments of this invention, the dyestuff precursor can be either N-methyl-3-formylcarbazole or N-ethyl-3-formylcarbazole. Any one of a number of organic photoconductive materials can be present in the reaction mixture during the synthesis of this polymeric dyestuff. Typical of such organic photoconductive materials include any of the polyvinylcarbazoles (e.g. poly(N-vinylcarbazole); poly-3-vinylcarbazole; poly-2-vinylcarbazole; poly-3-halo-substituted N-vinylcarbazole; and poly-3,6-dihalo-substituted N-vinylcarbazole).

#### DESCRIPTION OF THE INVENTION INCLUDING PREFERRED EMBODIMENTS

According to this process, triaryl methane dyestuffs are prepared by condensation-polymerization of at least one dye precursor compound of the formula:



wherein R is an alkyl of 1 to about 5 carbon atoms, in a solution comprising polyphosphoric acid and an organic polymeric photoconductive material. Subsequent to the formation of the triaryl methane dyestuff, the colored polymeric products thus obtained are separated from the acid and, thereafter, formed from a suitable solvent into a photoconductive imaging layer.

The dyestuff precursor compounds, namely the N-alkyl-3-formyl carbazoles, which can be used in this process can be readily prepared from commercially available materials by methods disclosed in the technical literature. Typical of the materials which are suitable in this regard include N-methyl-3-formyl carbazole, N-ethyl-3-formyl carbazole, N-propyl-3-formyl carbazole, N-butyl-3-formyl carbazole and N-pentyl-3-formyl carbazole. The concentration of precursor compound(s) used in such synthesis is based upon the relative concentration of acid and organic polymeric photoconductive materials present in the reaction mixture. Generally, good results are obtained wherein the concentration of precursor in the reaction mixture is in the range of from about 2 to about 50 parts by weight precursor per 100 parts by weight organic polymeric photoconductive materials.

The reaction medium employed in the condensation-polymerization of the above materials is polyphosphoric acid. It is generally preferable that such acid be fairly concentrated. The relative concentration of such acid in the reaction mass should be in the range of from about 5 to 50 times the weight of organic polymeric photoconductive materials used in said synthesis.

The third essential component of the reaction mass is an organic polymeric photoconductive material. Any of the materials heretofore described in the patent and technical literature are suitable for use in said synthesis. Typical of the materials which can be selected as the organic polymeric photoconductive component of the reaction mass include the polyvinylcarbazoles - e.g. poly(N-vinylcarbazole), poly(N-ethyl-3-vinylcarbazole), poly(N-methyl-3-vinylcarbazole), poly(N-ethyl-2-vinylcarbazole), poly(N-methyl-2-vinylcarbazole); poly(vinylpyrene); and poly(vinylpyrenal). It is not believed that the organic polymeric photoconductive component of the reaction mass is chemically altered during synthesis of the triaryl methane dyestuff. The organic polymeric photoconductive material and the dyestuff are, however, physically bound together during the condensation-polymerization of the precursor compound, thus, forming a complex wherein the photoconductive material and the sensitizer are intimately associated with one another.

Subsequent to the intimate admixture of the above components in their proper relative proportions, the reaction mass thus produced is agitated and heated. The time required to effect formation of the desired product will vary with the temperature used in carrying out this process and the nature of the product desired. It is apparent that at elevated temperatures, the condensation polymerization of the dyestuff precursor will occur at an accelerated pace. The degree of polymerization of the triaryl methane dye at a given temperature is controlled by the duration of the reaction interval. For example, where the polymerization condensation of the N-alkyl-3-formyl carbazole is allowed to proceed (at 60°C) for less than about 10 minutes, the product

will predominantly comprise a triaryl methane dye (nonpolymerized) having the following structural formula:



wherein X is an anion residue

Where the condensation polymerization is allowed to proceed for a more extended period of time the product thus produced will comprise a mixture of materials including the triaryl methane dye and the highly polymerized form of the dye having the following structural formula:



wherein X is an anion residue

Subsequent to preparation of the triaryl methane dye in the desired form (polymerized v. nonpolymerized) the reaction is quenched by pouring the reaction mass into a large volume of distilled water. The colored polymeric products precipitate out and are separated from the aqueous medium by filtration. Subsequent to removal of these aqueous residues the colored polymeric product is purified by reprecipitation from alternate solutions of water and methanol. After the colored polymeric products have been cleansed of impurities, it can be dissolved in a suitable solvent, such as chloroform or methylene chloride, and coated on a suitable conductive substrate (aluminized mylar, conductive glass plates, aluminum, etc.). The quantity of material which is imparted to such a substrate should be sufficient to form a photoconductive imaging film having a dry film thickness in the range of from about 0.5 to about 50 microns. It has been observed, that prior to casting of

such materials on the conductive substrate, preillumination of such materials in the casting solvent with activating electromagnetic radiation enhances the optical



density of the dissolved dyestuff.

The Examples which follow further define, describe and illustrate the process of this invention. Apparatus and techniques used in such process are presumed to be standard or as hereinbefore described. Parts and percentages appearing in such Examples are by weight unless otherwise indicated.



#### EXAMPLE I - V

A series of dyestuff sensitized photoconductive compositions are prepared from poly(N-vinylcarbazole) and N-ethyl-3-formyl carbazole. The exact proportion of these materials in each of the compositions is disclosed in Table I appearing immediately after the text of this Example. In each instance, the poly(N-vinylcarbazole) is initially dispersed in 50 grams phosphoric acid. N-ethyl-3-formyl carbazole is then added to the dispersion while the dispersion is continuously vigorously agitated. The temperature of this dispersion is gradually increased to about 60°C and thereafter maintained at this level for the prescribed reaction interval. At the end of the prescribed reaction interval, the reaction mass is poured into one liter of distilled water whereupon the colored polymeric products form a precipitate. The precipitate is then separated from the aqueous solution by filtration, dried under a

vacuum and thereafter dissolved in a suitable solvent (e.g. chloroform or methylene chloride). In a limited number of situations (Examples VIII and IX) the casting solvent containing the polymeric composition, is subjected to preillumination with activating electromagnetic radiation whereby its optical density is substantially enhanced. Subsequent to this preillumination treatment the solution containing the colored polymeric solids is cast or coated on an appropriate conductive substrate. The quantity of colored polymeric materials that is transferred to such substrates is sufficient to form a substantially uniform film having a thickness in the previously prescribed range. Any of the conductive substrates traditionally used in the preparation of electrophotographic imaging members are suitable.

TABLE I

| Example No. | Poly(N-vinyl carbazole) (g) | N-ethyl-3-formyl-carbazole (g) | Reaction time (minutes) | Absorption peak in nanometers (nm) |
|-------------|-----------------------------|--------------------------------|-------------------------|------------------------------------|
| I           | 2                           | 0.1                            | 10                      | 602                                |
| II          | 2                           | 0.1                            | 20                      | 609                                |
| III         | 2                           | 0.1                            | 60                      | 609                                |
| IV          | 2                           | 0.2                            | 60                      | 610                                |
| V           | 2                           | 0.4                            | 60                      | 610                                |

Reaction temperature 60°C in Examples I – V.

## EXAMPLE VI

About 0.2 grams of the colored polymeric composition of Example I is dissolved in 6 milliliters of methylene chloride and thereafter coated on a conductive paper substrate such that its dry film thickness is about 15 microns. Subsequent to curing of this polymer coating, the resulting imaging member is processed in a standard electrophotographic imaging system. The source of illumination used in projecting the image pattern on the corona sensitized polymeric coating is a tungsten lamp. The amount of exposure required to give what was deemed to be an image of good quality is 70 lux. seconds.

## EXAMPLE VII

The procedures of Example I are repeated except with the polymer composition of Example II. The latent electrostatic image formed on the surface of the imaging layer is rendered visible by development with a liquid developer composition comprising a dispersion of a commercially available black offset ink in a cyclohexane solution; the relative concentration of ink in the solvent being 1 gram per liter solvent. The duration of exposure required to obtain an image comparable to that of Example I is 68 lux. seconds.

## EXAMPLE VII

The procedures of Example VI are repeated with the colored polymeric composition of Example III. The amount of exposure required to obtain an image comparable to that of Example I is 53 lux. seconds. The action spectrum for the material used in preparation of the imaging layer of the imaging member used in this Example is shown in FIG. 1.

## EXAMPLE VIII

About 2 grams of the colored polymeric composition of Example IV is dissolved in about 1 milliliter of methylene chloride and the resulting solution subsequently irradiated from a distance of 30 centimeters with a fluorescent lamp (20 watts). The effects of such irradiation on a sample not having received such irradiation and samples irradiated for five minutes and 20 minutes respectively are shown in Table II.

TABLE II

| Sample No. | Time of irradiation (minute) | An amount of correct exposure for picture image (lux. second) |
|------------|------------------------------|---------------------------------------------------------------|
| A          | 0                            | 51                                                            |
| B          | 5                            | 47                                                            |
| C          | 20                           | 44                                                            |

It is clear that irradiation of the colored polymeric material prior to coating on the conductive substrate improves the sensitivity of such material to activating electromagnetic radiation.

## EXAMPLE IX

About 0.1 grams of the polymeric composition of Example IV and about 0.1 grams of poly(N-vinylcarbazole) are dissolved in 6 milliliters of methylene chloride. The resulting solution is subjected to irradiation in a manner similar to that of Example IX. Following irradiation, a conductive paper substrate is coated with said solution. Sufficient polymeric materials are transferred to the paper to provide a photoconductive imaging layer having a dry film thickness equal to about 15 microns. A comparative evaluation of the sensitivity of an irradiated sample with a non-irradiated sample are shown in Table III.

TABLE III

| Sample No. | Time of irradiation (minute) | An amount of correct exposure for picture image (lux. second) |
|------------|------------------------------|---------------------------------------------------------------|
| D          | 0                            | 68                                                            |
| E          | 10                           | 51                                                            |



What is claimed is:

1. A process for preparation of a dyestuff sensitized photoconductive composition from an organic polymeric photoconductive material, polyphosphoric acid and a compound of the formula



wherein R is alkyl of 1 to 5 carbon atoms, said process comprising:

- a. providing a mixture containing (i) organic polymeric photoconductive material (ii) about 2 to about 50 parts by weight of a compound of the

20

3. The process of claim 1, wherein the organic polymeric photoconductive material is poly(3-vinylcarbazole).

4. The process of claim 1, wherein the organic polymeric photoconductive material is poly(2-vinylcarbazole).

5. The process of claim 1, wherein the organic polymeric photoconductive material is poly(vinylpyrene).

6. The process of claim 1, wherein the organic polymeric photoconductive material is poly(vinylpyrenal).

10 7. The process of claim 1, wherein the compound of the above structural formula is N-methyl-3-formyl carbazole.

15 8. The process of claim 1, wherein the compound of the above structural formula is N-ethyl-3-formyl carbazole.

9. The process of claim 1, wherein heating of the mixture proceeds for an interval sufficient to produce a composition wherein the predominant component is

20 triaryl methane dyestuff of the formula



above formula per 100 parts organic polymeric photoconductive material, and (iii) a quantity of polyphosphoric acid equivalent to about 5 to about 50 times the weight of organic polymeric photoconductive material in the mixture; and

- b. heating said mixture at a temperature in the range of from about 20° to about 120°C for an interval sufficient to effect condensation polymerization of the compound of the above formula to the extent desired.

2. The process of claim 1, wherein the organic polymeric photoconductive material is poly(N-vinylcarbazole).

45 wherein X- is an anion residue and R is as previously defined.

10 10. The process of claim 1, wherein heating of the mixture proceeds for an interval sufficient to produce a composition wherein the predominant component is a polymeric triaryl methane dyestuff of the formula wherein X- is an anion residue and R is as previously defined

50 11. The process of claim 1 wherein a solution of the polymeric products of step (b) is exposed to activating electromagnetic radiation for a duration sufficient to enhance its optical density.

55

\* \* \* \* \*

UNITED STATES PATENT AND TRADEMARK OFFICE

**CERTIFICATE OF CORRECTION**

PATENT NO. : 3,895,945

DATED : July 22, 1975

INVENTOR(S) : Syu Watarai et al

It is certified that error appears in the above-identified patent and that said Letters Patent are hereby corrected as shown below:

Column 1, line 52, insert quotations around plain paper to make it read "plain paper".

Column 1, line 53, --prefereably-- should be "preferably".

Column 2, line 11, --2,4,7-trinitro-9-fluonone-- should be "2,4,7-trinitro-9-fluorenone".

Column 3, line 2, --pigment-- should be "pigment.".

Column 4, line 1, omit the period after atoms.

Column 4, line 27, --condensationpolymerization-- should be "condensation-polymerization".

Column 4, line 44, --poly(vinylpryene)-- should be "poly(vinylpyrene)".

Column 4, line 45, --poly(vinylpryenal)-- should be "poly(vinylpyrenal)".

Column 6, line 53, --senistized-- should be "sensitized".

Column 10, line 18, --predominent-- should be "predominant".

UNITED STATES PATENT AND TRADEMARK OFFICE  
CERTIFICATE OF CORRECTION

PATENT NO. : 3,895,945  
DATED : July 22, 1975  
INVENTOR(S) : Syu Watarai et al

It is certified that error appears in the above-identified patent and that said Letters Patent are hereby corrected as shown below:

Column 10, line 48, after the words "triaryl methane dyestuff of the formula", insert the following formula



Signed and Sealed this  
fourth Day of November 1975

[SEAL]

Attest:

RUTH C. MASON  
Attesting Officer

C. MARSHALL DANN  
Commissioner of Patents and Trademarks